

Sept. 6, 1927.

1,641,292

V. PLANCHON

MANUFACTURE OF NITRATED CELLULOSE FROM WOOD PULP

Filed Feb. 27, 1925

Fig.1



Fig.2



Fig.3



Inventor:

Victor Planchon

By *Samuel Nichols*  
Attorney.

Patented Sept. 6, 1927.

1,641,292

# UNITED STATES PATENT OFFICE.

VICTOR PLANCHON, OF LYON, FRANCE.

## MANUFACTURE OF NITRATED CELLULOSE FROM WOOD PULP.

Application filed February 27, 1925, Serial No. 12,170, and in France February 29, 1924.

Nitrated cellulose is obtained, in practice, by using cotton or thin paper treated according to the well-known nitration process. Attempts have been made to substitute for 5 cotton a less expensive raw material such, for instance, as wood pulp in sheets for example, but such attempts have hitherto proved fruitless and it is generally known that wood pulp is practically incapable of 10 being nitrated by the known methods owing to the fact that the sheets of wood pulp are hydrolyzed and partly dissolved long before the nitration is completed.

In the present invention, only wood pulp 15 in sheets is used to obtain nitrated cellulose.

The invention is characterized by the following points:

1. The usual nitration bath (a mixture of nitric acid and sulphuric acid) is used at a 20 temperature always below 15° C., and the sheets of wood pulp are immersed in the aforesaid bath for a sufficient period which depends on the temperature of such bath and which, consequently, varies with said 25 temperature.

2. A method of manufacture is used which is peculiar to the employment of wood pulp sheets for obtaining nitrated cellulose and which is altogether unsuitable for the ordinary manufacture of nitrated cellulose from 30 cotton, waste from spinning thin paper, etc.

In the annexed drawing:

Figure 1 is a perspective view, with parts 35 broken away, of a vat containing a support for the wood pulp sheets to be nitrated.

Fig. 2 is a perspective view of another device for maintaining the sheets a few millimeters apart in the bath.

Fig. 3 shows diagrammatically an apparatus for carrying out the process according 40 to the present invention.

The wood pulp sheets suitable for the manufacture are those which are found in commerce in the well-known form of thick 45 sheets similar to blotting paper and used in the manufacture of viscose. These sheets, of the size current in trade, are, first, placed in grooves of a support constructed of acid proof metal, such as aluminum, and capable 50 of being immersed with its contents in a vat filled with acids which compose the nitration bath.

The grooves of the support, which is similar 55 to that used for the vertical washing of photographic plates, are brought sufficiently close to one another to leave between the

sheets a space of a few millimeters only. A support of this character is illustrated in Fig. 1, and is generally designated 1, the grooves or seats 2 being formed in its upper 60 and lower horizontal members 3 and 4. The pulp sheets are designated 5 and the vat is designated 6.

The sheets of pulp may alternatively be 65 perforated at selected points of their surface as indicated at 7 in Fig. 2, and be placed in juxtaposition, strung one after another on glass rods 8 so that they may be separated by small spaces, as shown.

The unit made up in one or the other of 70 the two ways mentioned may consist of any number of sheets—for instance, 50 sheets weighing 100 grams each—and the nitration is effected afterwards simultaneously in the same vat on several units of this description, 75 say 6 for example, representing 30 kilograms of pulp which after nitration will yield, on an average, 50 kilograms of nitrocellulose.

The immersion vats 6 may be made of any 80 resisting metal but, as it is most important, from a hygienic point of view, to operate in closed vessels and therefore to carry out the first washing operations in the actual vat where the nitration takes place, preference is given to aluminum which is very resistant to 85 acids either concentrated or diluted with water. The shape and dimensions of these vats may vary, as may also the method of suspending the sheets.

By way of example, a construction suitable 90 for industrial manufacturing is represented in Fig. 3 which shows a rectangular vat A surrounded by a jacket B, through which a current of water at a constant temperature is continuously circulating, the vat 95 having its top part closed by a light and close-fitting cover C of the same metal.

When said vat is empty and the cover 100 raised, the free ends of the rods carrying the units are deposited on cross bars D D, the cover is fitted on, and the different valves with which the vat is externally provided 105 permit the nitration and the first washings being carried out hermetically. For this purpose, the valve E which regulates the influx of the nitrifying mixture supplied by the upper tank F, is opened. The liquid rises from the bottom of the vat and fills it to the level necessary to entirely immerse 110 the pulp sheets; such level being reached when it is observed from outside that the intermediate funnel G begins to be filled. At

that moment valve E is closed and the nitration proceeds.

During nitration, the circulation of the water is maintained in the jacket B. The 5 temperature of the refrigerating water should only vary within very narrow limits (1 or 2 degrees, for instance); it must not appreciably exceed 15° C. This condition, which is indispensable to insure the success 10 of the operation, is easily realized by employing an intermediate vat in which the spring and well water etc., used may be cooled by a circulation of brine obtained from any refrigerating apparatus.

15 The nitration is thus carried on at a constant temperature without any need to raise the cover of the vat, but its duration cannot be predetermined because it depends upon the composition and temperature of the nitration bath employed.

20 It is known that the nitrocellulose obtained has a substantially-constant percentage of nitrogen when the bath used is itself constant. This is why, in order to prepare 25 the variety of soluble nitrocellulose called "collodion quality" with 10 or 10.5% of nitrogen, the nitration bath must, for instance, contain:

|    |                                |     |
|----|--------------------------------|-----|
| 30 | H <sub>2</sub> SO <sub>4</sub> | 62% |
|    | HNO <sub>3</sub>               | 20% |
|    | H <sub>2</sub> O               | 18% |

35 If a bath of this description is used, the total nitration of the wood pulp will require about 12 hours if the operation is carried on at a temperature of 15° C., and about 20 hours at 10-11°.

40 With these temperatures, the nitration proceeds gradually and smoothly. It may be checked by testing specimen sheets taken, say, every hour. The percentage of nitrogen and the increase in weight of said sheets may be expressed by curves. Such curves are regular and at the end of the period 45 above-mentioned they become asymptotic, showing that the maximum of nitration has been reached.

50 A longer treatment, even extending to many hours, does not appreciably alter either the percentage of nitrogen or the weight of the nitrated product.

55 Unlike the violent reactions occurring in nitration in drying machines, a considerable margin of time remains available which makes it possible to work steadily and to carry out, if necessary, in the course of working any test considered necessary. Such margin of time is greater, as the bath is colder. But it is advisable not to prolong the period of nitration unreasonably and to fix a maximum period of 24 hours, and for this purpose to maintain the requisite temperature of the refrigeration water.

60 The use of acid mixtures of suitable composition makes it possible to obtain from the

wood pulp other varieties of nitrocellulose with the same facility as the "collodion quality," including explosives containing 13% of nitrogen. The quantities yielded do not appreciably differ from those obtained 70 with cotton.

75 After the nitration and without removing the cover, the bath, after use, is evacuated by opening the outlet valve L. The acid mixture passes through the pipe M into the tank N provided underneath. Said bath is afterwards analyzed, recharged with fresh acids and conveyed by means of an elevator to the initial tank F to serve for a further 80 operation.

85 When the vat is empty, about half an hour is allowed to elapse to permit the sheets of nitrated pulp to completely drain off, valve L is then closed and the washing is started. The washing water is supplied through the pipe O controlled by the valve P, fills up the tank, meets the overflow R and runs over into the drain pipe. This lixiviation is carried on until the evacuated water shows no appreciable acidity. The 90 washing is stopped by closing the valve P and the vat is emptied by opening the valve S.

95 The nitration operation is then completed. The cover C is removed and the parcels of sheets are withdrawn either with their grooved supports or with the aid of the glass rods upon which said sheets are suspended. The vat thus emptied may at once be used 100 again for a fresh operation.

105 The nitrated sheets are then transported to the finishing workshop and placed, assembled together as they are, in wooden tanks or vats of a large size for the purpose of being therein stabilized, modified (as regards the viscosity of the solutions they are to supply afterwards), bleached and thoroughly re-washed, being immersed vertically in the various baths in the same way as during nitration.

110 The wonderful consistency of the sheets of nitrated woodpulp enables them to stand a very long contact even with boiling baths. They are very easily manipulated with their supports up to the final drying which is effected either in a stove in vacuo or in any suitable dryer. After drying, the sheets are finally removed from their supports, cut and packed in any dimensions as in the case of ordinary cardboard.

115 If it is desired to keep the sheets in a moist condition, they are arranged in regular piles which are subjected to the action of a press for the purpose of squeezing out of them the water in excess before packing 125 them. The moist sheets may also be reduced to small fragments by subjecting them to the rapid action of known rotary crushers, which at once transform them into a light pulp.

As has already been stated, the process above described consists of operations entirely different from those which are generally followed in the case of cotton, lint, spinning noils, thin paper, etc., now used for the industrial manufacture of nitrocelluloses. It does away with the very dangerous and unhealthy use of nitration drying machines and requires neither heaters with acids, circulation piles nor dehydration turbines.

The sheets of wood pulp immersed in any liquid retain after draining very little of this liquid as compared with the quantities absorbed by cotton under the same circumstances. This is why special drying may be done away with and replaced by simple draining carried out, in the case of acids, in closed vessels.

To these advantages are added the low price of the raw material.

I claim as my invention:—

1. A process for manufacturing nitrated cellulose from wood pulp, comprising the steps of immersing thick wood-pulp sheets of low porosity in a nitration bath the temperature of which is below 15° C. but not less than 5° C., and maintaining said bath at a constant temperature during the whole period of nitration, such period varying according to the temperature of the bath.

2. A process for manufacturing nitrated cellulose from wood pulp, comprising the steps of immersing thick wood-pulp sheets of low porosity in a nitration bath the temperature of which is below 15° C. but not less than 5° C.; maintaining said sheets entirely free from contact with one another during their stay within the bath so as to enable the bath liquid to have free and uninterrupted access to all parts of them; and maintaining the bath itself at a constant temperature during the whole period of nitration, such period varying according to the temperature of the bath.

3. A process for manufacturing nitrated cellulose from wood pulp, comprising the steps of immersing thick wood-pulp sheets of low porosity in a nitration bath contained in a closed vessel, the temperature of such bath being below 15° C. but not less than 5° C.; maintaining said bath at a constant temperature during the whole period of nitration, such period varying according to the temperature of the bath; evacuating the bath liquid from said vessel at the conclusion of nitration, and leaving the nitrated sheets therein to drain; and then washing the drained sheets in said vessel with water.

In witness whereof I have signed this specification.

VICTOR PLANCHON.